

No. 832,605.

PATENTED OCT. 9, 1906.

G. W. GENTIEU.  
MANUFACTURE OF EXPLOSIVES.  
APPLICATION FILED MAY 10, 1906.



Witnesses:

E. W. Giles

Mary E. Conroy

Inventor.

George W. Gentieu  
By J. M. T. Giff

Atty.

# UNITED STATES PATENT OFFICE.

GEORGE W. GENTIEU, OF PEORIA, ILLINOIS.

## MANUFACTURE OF EXPLOSIVES.

No. 832,605.

Specification of Letters Patent.

Patented Oct. 9, 1906.

Application filed May 10, 1906. Serial No. 316,166.

*To all whom it may concern:*

Be it known that I, GEORGE W. GENTIEU, a citizen of the United States, residing at Peoria, in the county of Peoria and State of Illinois, have invented certain new and useful Improvements in the Manufacture of Explosives; and I do hereby declare that the following is a full, clear, and exact description of the invention, which will enable others skilled in the art to which it appertains to make and use the same.

This invention has reference more particularly to the manufacture of smokeless powder; and my object is to provide a process for producing a smokeless explosive which is superior to those obtained by the present processes.

Smokeless powder is made chiefly from nitrocellulose, and if it is necessary, particularly in ordnance-powder, that it have a high degree of elasticity and toughness, so as to withstand the enormous pressure to which it is subjected in the powder-chamber during the firing of the charge. The rate of burning or rapidity of the explosion of the powder depends on the size of the powder grains and the consequent burning-surface of the powder, the powder for the various sizes of guns being made in grains or sticks of suitable size to retard the explosion somewhat and generate gas just fast enough to exert a gradually-increasing pressure on the projectile and gradually overcome the inertia of the projectile to be thrown by that particular gun. If the grains or sticks of explosive are brittle or lack sufficient toughness and elasticity to withstand the pressure to which they are subjected during the explosion of the charge, they are broken up into fragments by the pressure, thus increasing the burning-surface, and consequently the rapidity of the explosion, which results in the transformation of the complete charge of powder into gas before the inertia of the projectile is overcome and a large enough chamber formed to accommodate the increased volume of gas and creates a pressure which the walls of the rifle are unable to withstand and bursts the gun or severely strains it.

Nitrocellulose, which, as has been hereinbefore suggested, is commonly used as the basis for smokeless powder, is made chiefly from cotton, as it is the purest and most satisfactory form of cellulose. The cotton consists of long tubular fibers or hollow cells, and its hollow cellular structure is not destroyed

or noticeably impaired by the process of nitrocellulose, the tubular or hollow cellular structure being retained in the nitrocellulose. In the manufacture of powder from the nitrocellulose it is first pulped and thoroughly cleansed from acid, then dehydrated and colloided to such a consistency that it can be granulated or pressed into sticks or pellets, and I have found that if the initial hollow cellular structure of the nitrocellulose is retained throughout the process of manufacture of smokeless powder therefrom a powder of great elasticity and toughness is obtained. The processes at present used in the manufacture of powder from nitrocellulose are accompanied with more or less stirring and compressing action, which breaks up the hollow cellular structure of the nitrocellulose and results in the production of a powder that is somewhat brittle and of insufficient elasticity and toughness to withstand the pressure of the explosion in the powder-chamber.

In my process I provide a method of treatment of the nitrocellulose whereby it can be made into powder without any stirring or compression, thus enabling me to retain the original cellular structure of the nitrocellulose and produce a powder of great elasticity and a high degree of toughness.

It is customary to colloid the nitrocellulose by mixing therewith alcohol and ethyl ether, neither of which said liquids is in itself a solvent of nitrocellulose, but which when combined in suitable proportions form a solvent. The usual method employed to mix the alcohol and ether with the nitrocellulose is to take nitrocellulose while wet from the cleansing or washing process, compress the same in the cylinder of a press, and displace the water remaining therein with alcohol by percolation, which reduces the nitrocellulose to the form of a hard compact block. Then take the alcoholized nitrocellulose from the cylinder of the press, break it up into small particles, and mix with it a suitable quantity of ethyl ether to combine with the alcohol and form a solvent and gelatinize the nitrocellulose.

In my process, which relates more particularly to the method of mixing the ether with the alcoholized nitrocellulose, I prefer to use nitrocellulose which has been dehydrated and alcoholized by the centrifugal wringer process set out in an application for patent for a dehydrating process, filed by me April

27, 1906, Serial No. 314,010. In this process the wet nitrocellulose is introduced into the interior of a centrifugal wringer which is revolved at a high rate of speed and removes 5 the greater per cent. of the water from the nitrocellulose and mats it against the perforated wall of the wringer. After the surplus water has been removed from the nitrocellulose, alcohol or other suitable liquid is 10 sprayed against the inner surface of the mass of nitrocellulose and as the wringer continues to revolve forces its way through the mass of nitrocellulose, thereby displacing the water therein and leaving the nitro- 15 cellulose saturated with alcohol. I prefer the above process, as the cellular structure of the nitrocellulose is not impaired thereby and it retains its light porous condition and is better adapted to absorb the ether-vapor. 20 However, I do not confine myself to nitrocellulose treated by my foregoing process, but take nitrocellulose treated by any suitable process which contains the required amount of alcohol, place it in wire-mesh or other 25 suitable trays which will readily permit the entrance of ether-vapor to all parts of the nitrocellulose contained therein, and place the trays of nitrocellulose in a suitable receptacle or oven which is practically air-tight. 30 Ether is then introduced into a pan or other suitable container within the oven and allowed to evaporate or vaporize, the oven or receptacle being kept at a sufficient temperature (about 30° centigrade) to vaporize the ether slowly without boiling. The 35 nitrocellulose being wet with the proper per cent. of alcohol has the property of absorbing the ether-vapor very readily, which said vapor combines with the alcohol in the nitrocellulose and forms a solvent which gelatinizes the nitrocellulose. As is apparent, by regulating the time and the amount of ether and alcohol used the nitrocellulose may be colloided to the required degree. 40 After the material has been colloided to the required degree it is taken from the oven and is ready to be pressed out into powder grains. Before being pressed into powder grains it may, however, if desired, be run through a screening-press or passed between a pair of rolls to remove any lumps. This powder when dried will be found to be much tougher and less brittle than that made by processes wherein the nitrocellulose is subjected to any stirring or compressing action, which quality is due to the fact that the original hollow cellular structure of the nitrocellulose has not been destroyed or noticeably impaired by my process.

In order that my process may be more clearly understood, I have illustrated in the accompanying drawings an apparatus such as I prefer to employ for carrying out my process, and I will now describe my process in connection therewith.

In said drawings, Figure 1 is a vertical longitudinal sectional view of the apparatus, and Fig. 2 is a vertical cross-sectional view of the apparatus on the line *a-a* of Fig. 1 looking as indicated by the arrow.

1 is an oven or receptacle which is built with hollow walls, which are formed of the inner and outer casings 2 and 3, suitably spaced apart and held together by means of the rivets 4. The hollow walls of the oven 75 or the space between the inner and outer casings 2 and 3 is designed to be filled with water to keep the oven at an even temperature, and there is provided an inlet-pipe 5 at the top of the oven and an outlet-pipe 6 at 80 the bottom of the oven, whereby hot water may be circulated through the hollow walls of the oven. For the purpose of indicating the temperature of the water that is introduced into the oven there is provided a thermometer 7, suitably fixed in the inlet-pipe 5.

In the bottom of the oven or receptacle 1 is a shallow pan 8, which is used to contain the ether which is evaporated in the process of gelatinizing the nitrocellulose, the ether 90 being supplied to said pan from the tank 9 through the supply-pipe 10 and control-valve 11. This ether-tank 9 is provided with any suitable means for filling the same, such as a common opening in the top thereof, closed by the threaded plug 12, and there is provided at the side of the tank a graduated gage-glass 13, whereby the amount of ether used may be regulated.

For the purpose of allowing access to the 100 interior of the oven one end thereof is provided with a large opening 14, which is adapted to be closed practically air-tight by means of the door 15. This door may be constructed to slide in ways 16 or otherwise adapted to 105 be moved free of the opening 14.

17 represents wire-mesh trays or baskets for holding the nitrocellulose, the said trays being of such size that when inserted in the oven, as shown in the drawings, there will be a 110 circulating-space between the said trays and the oven-wall, and said trays are furnished with handles 18 to hold the trays a suitable distance apart and provide a circulating-space between them and for the purpose of 115 convenience in handling. These trays are preferably mounted on small truck-wheels 19, which travel on the tracks 20, located at each side of the bottom of the oven, so that the trays may be readily carried in and out of said 120 oven.

In using the apparatus just described to carry out my process the trays 17 are filled with nitrocellulose 21 which has been dehydrated by any wet process, preferably by 125 my centrifugal wringer process hereinbefore mentioned, and which contains a certain percentage of liquid which is not in itself the solvent for nitrocellulose, in this case alcohol being the liquid specified. These trays are 130

then placed in the oven 1 and the door 15 thereof closed, so as to keep the compartment or oven practically air-tight. Ether is then introduced into the evaporating-pan 8 from the ether-tank 9, the amount used being indicated by the gage-glass 13, thus enabling the operator to introduce a sufficient quantity into the evaporating-pan to colloid the nitrocellulose to the proper degree. Water is circulated in the hollow walls of the oven to keep the oven at a suitable temperature to vaporize the ether without boiling, and as the ether evaporates and circulates in the oven it is readily absorbed by the wet nitrocellulose in the trays 17. When the proper amount of ether has been evaporated in the oven to colloid the mass of nitrocellulose, the nitrocellulose is removed from the oven and may be pressed directly into powder or may be first passed through a screening-press or between a pair of rollers in order to blend the mass and remove any lumps.

If it is desired to produce a granulated explosive for small-arms, the colloided material may be transferred to any suitable receptacle provided with a propeller or movable arms and blades and rapidly agitated, which operation breaks the mass of colloided nitrocellulose into small grains or granules, which are then removed to a suitable solvent-recovery apparatus, the solvent recovered, the grains dried and sifted, when they will be found to form a smokeless powder of high quality.

I am aware of Letters Patents Nos. 430,212 and 436,898, granted to Hiram Stevens Maxim, wherein a process is set out for colloiding

nitrocellulose by subjecting it to vapor of a solvent. In these processes, however, the nitrocellulose is used in a dry state and subjected to the solvent-vapor in a vacuum. In my process, however, I use nitrocellulose in a wet state, as it absorbs the vapor more readily and evenly, and I do not use the vacuum.

I have described my process particularly with reference to the process of subjecting alcoholized nitrocellulose to ether-vapor; but the method may be reversed—that is, nitrocellulose which is saturated with ether may be subjected to alcohol-vapor or other liquids may be employed without departing from the spirit of my invention.

What I claim is—

1. The process of colloiding nitrocellulose which consists in mixing with the nitrocellulose a liquid which is not in itself a solvent of the nitrocellulose, then subjecting the wet nitrocellulose to a vapor which combines with the liquid in the nitrocellulose and forms a solvent thereof.

2. The process of colloiding nitrocellulose which consists in mixing alcohol with nitrocellulose, then subjecting the alcoholized nitrocellulose to ether-vapor which combines with the alcohol in the nitrocellulose and forms a solvent thereof.

In testimony whereof I have affixed my signature in presence of two witnesses.

GEORGE W. GENTIEU.

Witnesses:

E. M. GILES,  
MARY E. COMEGYS.